

April 1, 1947.

M. R. HUTCHISON

2,418,304

ADHESIVE PHOTOSENSITIVE MATERIAL

Filed Dec. 22, 1943



INVENTOR

MILLER REESE HUTCHISON

BY

*Morrison Kennedy Campbell*  
ATTORNEYS

## UNITED STATES PATENT OFFICE

2,418,304

## ADHESIVE PHOTORESITIVE MATERIAL

Miller Reese Hutchison, New York, N. Y., assignor, by mesne assignments, to Ralph G. Luff, Philadelphia, Pa.

Application December 22, 1943, Serial No. 515,282

2 Claims. (Cl. 95—8)

1

In my Patent No. 2,311,547, granted February 16, 1943, I have disclosed a process for producing templates and the like, which process includes the preparation of three different laminated units, each comprising a substantially rigid backing element, which is non-hygrosopic in character, and a surface layer of sheet material (paper), which, though hygroscopic in character, is rendered immune to plane dimensional variations, regardless of moisture conditions, by being bonded to said rigid non-hygrosopic backing element, by means of a water-proof heat-setting adhesive. The first unit is the image or drawing unit, consisting of a metal backing element, surfaced with plain paper, on which the template design is drawn in pencil. The second unit is the negative unit, consisting of a glass backing element, surfaced with photographic paper, on which a reflex negative is produced from the drawing unit. The third unit is the positive unit, consisting of a metal backing element, surfaced with photographic paper, on which a positive print is made from the reflex negative unit, said metal backing element becoming the finished template after being machined in accordance with the template design, reproduced thereon.

The photographic paper, employed for the negative and positive units, is prepared in the usual way; that is to say, by looping the paper transversely and drawing it over the surface of an aqueous photographic emulsion solution and then leading the coated paper over a roller past a "doctor bar" located at a fixed distance from the surface of the paper, whereby an emulsion coating, of a definite uniform thickness, is produced on the paper. The coating of the water-proof heat-setting adhesive is applied to the paper in the same way, the coating being applied in liquid or solution form. In each instance, after the application of the coating, the paper is led through a drying alley for a period of time long enough to dry and to solidify the applied coating. In my prior patent, the described procedure contemplates the application of the adhesive coating prior to the application of the emulsion coating, it being thought, at the time, that, by following such sequence, it would be easier to apply the emulsion coating, because of the stiffening of the paper produced by the previously applied adhesive coating.

As thus prepared, the photographic paper is laid with its adhesive face in contact with the surface of the backing element, to which it is to be applied (glass in one instance and metal in the other), and then bonded to the backing element, under heat and pressure. However, in my prior

2

patent, the adhesive coating on the photographic paper is not relied upon alone for bonding the paper to the backing element, but the latter itself is first prepared with an adhesive coating for contact with the adhesive coating of the paper, it being thought, at the time, the two coated surfaces would produce a firmer bond than could be secured if only one of the two surfaces were coated.

10 As explained in my prior patent, the adhesives employed must have special characteristics. Thus, for the positive laminated unit, the adhesive must be such that, when the photographic paper is bonded to the metal backing element, by 15 the heat-setting of the adhesive, said bond will be unaffected by the heat generated during the template machining operations, which may develop a temperature of between 500° F. and 600° F., and, in addition, the adhesive must be sufficiently water-proof, dilute-acid-proof and dilute-alkali-proof that, when the photographic paper is bonded to the backing element, by the heat-setting of the adhesive, said bond will be unaffected by the solutions used in the processing 20 of the photographic emulsion, after the printing exposure. For the negative laminated unit, the adhesive must likewise be sufficiently water-proof, dilute-acid-proof and dilute-alkali-proof that, when the photographic paper is bonded to the 25 glass backing element, by the heat-setting of the adhesive, said bond will be unaffected by the solutions used in the processing of the photographic emulsion, after the printing exposure; and, moreover, the adhesive, once heat-set, must possess 30 the requisite light-transmitting properties. The adhesive for the negative laminated unit should also, preferably, be of such character that the bond between the photographic paper and the glass backing element may be broken, either by 35 prolonged water soaking or by the use of solvents of the adhesive, in order that the same glass backing element may be used over and over again in making reflex negatives. However, it is to be 40 noted that, regardless of the characteristics mentioned, the adhesives must be of the heat-setting variety (whether thermo-plastic or thermo-setting or both), no cold-setting adhesive having 45 been found which would answer the requirements.

My present invention is concerned solely with 50 the preparation of the negative and positive laminated units, presenting an improved adhesive photographic paper, suitable for the purpose.

As one feature of my invention, I have discovered that better results may be obtained by 55 omitting the adhesive coating from the backing element and applying an adhesive coating only to

the photographic paper. By doing this, I find that I not only obtain an adhesive coating of uniform thickness, which is most desirable, but, in addition, a coating of extreme thinness, e. g., .001" or even less, which also is most desirable. 5

As another feature of my invention, I have also discovered that better results may be obtained by first applying the emulsion coating to the paper base and causing it thoroughly to dry or solidify, then applying the adhesive coating to the paper 10 base and causing it thoroughly to dry or solidify, and finally rolling up the double-coated paper with the adhesive face in direct contact with the emulsion face.

In following the procedure described in my 15 issued patent, I found that, when the adhesive coating is first applied to the paper base, the coated paper, unless prevented from doing so, will curl or assume a tube-like form when the paper loop is moved into and out of contact with the surface of the emulsion in the applying trough. This curling or tubing effect is probably caused by the water-proof character of the already applied and solidified adhesive coating, on one side of the paper, and the non-water-proof or water-absorbing character of the opposite or emulsion-taking side. In other words, when the emulsion coating is applied, the paper will absorb water from the highly aqueous emulsion solution and expand on one side, as it is free to do, but, because of the presence of the water-proof adhesive coating, the paper cannot expand on the other side. Hence, it became necessary to use mechanical means to hold the paper straight, as it is drawn through the emulsion trough and later through the long drying alley—a very difficult operation and one which is far from satisfactory.

This difficulty of curling does not arise when, according to the present invention, the emulsion coating is applied and dried before the application of the adhesive coating. The explanation seems to be that, in applying the emulsion coating onto plain or unlacquered paper, any expansion of the paper by water absorption from the aqueous emulsion solution is uniform throughout, and that, when the adhesive coating later is applied, no water is absorbed by the paper, due to the non-aqueous character of the adhesive solution, and hence no expansion of the paper takes place.

As another feature of the invention and one of great importance, I have discovered that, by the reverse sequence above described, the emulsion coating will not be fogged or otherwise contaminated by the adhesive coating, either during or after the coating step. In other words, I have discovered that, whereas the emulsion coating, before it becomes dried or solidified, is susceptible to fogging or contamination by the previously applied adhesive coating, the emulsion coating has no such susceptibility, in its dried or solidified condition. The explanation is probably this: If the emulsion coating is applied after the adhesive coating, the emulsion solution (being highly aqueous) penetrates through the paper stock and (being most sensitive) has a fair chance of being chemically affected by the already applied adhesive coating, both during the coating period and the slow drying period. On the other hand, if the adhesive coating is applied after the emulsion coating, the dried or solidified emulsion is absolutely impervious to the solvents used in preparing the adhesive solution, and this, whether the solvents are present in liquid or vapor form during the coating and drying periods.

When the adhesive photosensitive material is prepared in accordance with my present invention, the adhesive and emulsion coatings may be brought into direct contact, without any deleterious effect, in winding up the material into a roll, no liner or separator being needed. This, of course, is an added advantage of considerable importance from a practical standpoint.

I should, perhaps, add that the photographic emulsion which is employed, in the practice of my present process, is the same as that described in my prior patent above identified. In other words, the emulsion solution is prepared so that the emulsion coating of the photographic paper, as used for both the negative and positive units, will have an initial sensitivity greater than that required for the service intended, so as to compensate for whatever loss of sensitivity takes place in the heat-setting of the adhesive and subsequent conditioning when the photographic paper is bonded to the backing element. Notwithstanding such supersensitivity of the photographic emulsion, my present process of applying the emulsion coating first and the adhesive coating last, avoids any fogging or contamination of the emulsion, either during the coating and drying periods or, later on, during the plasticizing or heat-setting period.

Referring now to the drawings:

30 Fig. 1 is a sectional view, greatly enlarged, depicting a portion of a sheet of adhesive photosensitive material as prepared for making up the negative laminated unit. The material consists of a paper base 1 (about .003" in thickness) having, on one side, a uniform coating 2 (of the usual thickness) of an unexposed light-sensitive emulsion and, on the other side, a uniform coating 3 (about .001" in thickness) of a water-proof heat-setting adhesive, these coatings possessing the characteristics and being applied in the manner above described.

35 Fig. 2 is a sectional view, greatly enlarged, depicting the adhesive photosensitive material of Fig. 1 bonded, by the heat-setting of the adhesive coating, to a glass backing element 4 (about .25" in thickness as to template sizes up to 4' x 6' and thicker for larger ones), this paper-surfaced glass element being the laminated unit which is used in making a reflex negative print from the original drawing unit.

40 Fig. 3 is a sectional view, greatly enlarged, depicting a portion of a sheet of adhesive photosensitive material, as prepared for the making up of the positive laminated unit. The material consists of a paper base 5 (about .003" in thickness) having, on one side, a uniform coating 6 (of the usual thickness) of an unexposed light-sensitive emulsion and, on the other side, a uniform coating 7 (about .001" in thickness) of a water-proof heat-setting adhesive, these coatings possessing the characteristics and being applied in the manner above described.

45 The sheet of adhesive photosensitive material is bonded, by the heat-setting of the adhesive, to a metal backing element 8 (about .065" in thickness as to normal sized templates), this paper-surfaced metal element being the laminated unit which is used in making a positive print from the reflex negative print of Fig. 2 and which, as before explained, is later converted, by machining, into the final template.

50 Having thus described my invention, what I claim is:

55 1. As an article of manufacture, adapted for use in a photographic process for producing on a surface of the material to be fabricated an

accurate replica of some particular image, a laminated unit comprising a glass backing element and a photosensitive material adhered thereto, said photosensitive material comprising a flexible sheet material coated on one side with a first-applied unexposed light-sensitive photographic emulsion, and on the other side with a later-applied water-proof heat-setting adhesive, said photographic emulsion being immune to contamination by said adhesive, the heat-setting of the adhesive in bonding the sheet material to the glass backing element having the effect of reducing the sensitivity of the photographic emulsion, and the initial sensitivity of the emulsion being sufficiently greater than that necessary for the service intended to compensate for said reduction in sensitivity.

2. As an article of manufacture, adapted for use in the fabrication of a template or the like suitable for metal working operations, a laminated unit comprising a metal backing element possessing the requisite thickness and rigidity to become the finished template and capable of being machined in accordance with the template design, and a photosensitive material adhered thereto for the reproduction of the template design thereon, said photosensitive material com-

prising a flexible sheet material having one surface coated with a first-applied unexposed light-sensitive photographic emulsion and having its opposite surface coated with a later-applied water-proof heat-setting adhesive, said photographic emulsion being immune to contamination by said adhesive, the heat-setting of the adhesive in bonding the sheet material to the metal backing element having the effect of reducing the sensitivity of the photographic emulsion, and the initial sensitivity of the emulsion being sufficiently greater than that necessary for the service intended to compensate for said reduction in sensitivity.

15

MILLER REESE HUTCHISON.

## REFERENCES CITED

The following references are of record in the file of this patent:

## UNITED STATES PATENTS

| Number    | Name      | Date           |
|-----------|-----------|----------------|
| 770,421   | Derepas   | Sept. 20, 1904 |
| 1,605,699 | Bourges   | Nov. 2, 1926   |
| 2,147,772 | Kallander | Feb. 21, 1939  |
| 2,000,528 | Linderman | May 7, 1935    |

20

25